



US008282877B2

(12) **United States Patent**  
White et al.

(10) **Patent No.:** US 8,282,877 B2  
(45) **Date of Patent:** Oct. 9, 2012

(54) **PROCESS OF MAKING A HYDROENTANGLED PRODUCT FROM CELLULOSE FIBERS**

(75) Inventors: **Pat White**, Leics (GB); **Haio Harms**, Gmunden (AT); **Malcolm Hayhurst**, Bulkington (GB)

(73) Assignee: **Lenzing Aktiengesellschaft**, Lenzing (AT)

(\*) Notice: Subject to any disclaimer, the term of this patent is extended or adjusted under 35 U.S.C. 154(b) by 637 days.

(21) Appl. No.: **12/298,079**

(22) PCT Filed: **Apr. 26, 2007**

(86) PCT No.: **PCT/AT2007/000192**

§ 371 (c)(1),  
(2), (4) Date: **Mar. 11, 2009**

(87) PCT Pub. No.: **WO2007/124521**

PCT Pub. Date: **Nov. 8, 2007**

(65) **Prior Publication Data**

US 2009/0186189 A1 Jul. 23, 2009

(30) **Foreign Application Priority Data**

Apr. 28, 2006 (AT) ..... A 728/2006

(51) **Int. Cl.**

**B32B 3/10** (2006.01)  
**D01D 5/06** (2006.01)  
**D01D 5/12** (2006.01)  
**D01F 2/02** (2006.01)  
**D04H 3/08** (2006.01)

(52) **U.S. Cl.** ..... **264/555**; 28/104; 156/244.27; 156/324; 264/103; 264/132; 264/154; 264/187; 264/203; 264/210.2; 264/210.6; 264/210.8; 264/211.12; 264/211.14

(58) **Field of Classification Search** ..... 264/103, 264/187, 203, 210.8, 211.12, 211.14, 555, 264/132, 154, 210.2, 210.6; 156/244.27, 156/324; 28/104

See application file for complete search history.

(56) **References Cited**

U.S. PATENT DOCUMENTS

6,197,230 B1 3/2001 Pierre et al. ..... 264/6  
2002/0148050 A1 10/2002 Luo et al. ..... 8/115.51  
2004/0099981 A1 5/2004 Gerking ..... 264/103

2005/0035057 A1 2/2005 Zikeli et al. ..... 210/602  
2005/0056956 A1 3/2005 Zhao et al. ..... 264/37.24  
2005/0197028 A1 9/2005 Hartgrove et al. ..... 442/408

FOREIGN PATENT DOCUMENTS

|    |                   |           |
|----|-------------------|-----------|
| DE | 101 40 772 A1     | 3/2003    |
| EP | 1 358 369 B1      | 11/2003   |
| EP | 1 362 935 A1      | 11/2003   |
| EP | 1 614 790 A1      | 1/2006    |
| GB | 2 309 466 A       | 1/1996    |
| GB | 2337957 A         | * 12/1999 |
| WO | WO 95/35043       | 12/1995   |
| WO | WO 95/35399       | 12/1995   |
| WO | WO 95/35400       | 12/1995   |
| WO | WO 96/13071       | 5/1996    |
| WO | WO/97/19213       | 5/1997    |
| WO | WO 97/24476       | 7/1997    |
| WO | WO 98/07911       | 2/1998    |
| WO | WO 98/26122       | 6/1998    |
| WO | WO 99/47733       | 9/1999    |
| WO | WO 99/64649       | 12/1999   |
| WO | WO 01/88266 A1    | 11/2001   |
| WO | WO 03/056088 A1   | 7/2003    |
| WO | WO 2004/053216 A1 | 6/2004    |
| WO | WO 2005/106085 A1 | 11/2005   |
| WO | WO 2006/013378 A1 | 2/2006    |
| WO | WO 2006/035458 A1 | 4/2006    |
| WO | WO 2007/000319 A1 | 1/2007    |
| WO | WO 2007/022552 A1 | 3/2007    |

OTHER PUBLICATIONS

PCT Notification Concerning Transmittal of International Preliminary Report of Patentability (Chapter I of the Patent Cooperation Treaty) (Form PCT/IB/326); PCT International Preliminary Report on Patentability (Form PCT/IB/373); PCT Written Opinion of the International Searching Authority (Form PCT/ISA/237), (Aug. 30, 2007).

\* cited by examiner

*Primary Examiner* — Leo B Tentoni

(74) *Attorney, Agent, or Firm* — Fitzpatrick, Cella, Harper & Scinto

(57) **ABSTRACT**

The present invention relates to a process for the production of a hydroentangled product comprising cellulose fibers, which includes the steps of

- (a) extruding a solution comprising cellulose dissolved in an aqueous tertiary amine-oxide through a spinneret into an air gap, thereby forming filaments
- (b) drawing said filaments by means of a gaseous stream
- (c) collecting and precipitating said filaments in order to form a web
- (d) bonding said web by means of a hydroentanglement process
- (e) contacting said filaments in the air gap with a medium which at least partially coagulates the filaments.

Furthermore, the invention relates to products obtainable by said products, and uses thereof.

17 Claims, No Drawings

## 1

**PROCESS OF MAKING A  
HYDROENTANGLED PRODUCT FROM  
CELLULOSE FIBERS**

**CROSS-REFERENCE TO RELATED  
APPLICATIONS**

This application claims priority to International Patent Application No. PCT/AT2007/000192, filed Apr. 26, 2007, which claims priority to Austrian Patent Application No. A728/2006, filed Apr. 28, 2006.

**FIELD OF THE INVENTION**

The present invention relates to a hydroentangled cellulose product comprising cellulose fibers, processes for making the same, and uses thereof.

**BACKGROUND OF THE INVENTION**

It is known to produce nonwoven webs by so-called "melt-blown" processes from various synthetic polymers.

It is, furthermore, known to produce nonwoven webs made by a melt-blown process employing a cellulose solution in N-methyl-morpholine-N-oxide ("NMMO") from, inter alia, WO 98/26122, WO 99/47733, WO 98/07911, U.S. Pat. No. 6,197,230, WO 99/64649, WO 05/106085 and EP 1 358 369. Such products are also generally mentioned in DE 101 40 772 A1 and in WO 2007/000319 A1.

The melt-blown processes disclosed in the above-referenced documents are characterized in that extruded threads of the cellulose solution in NMMO are picked up by a gas stream flowing in a generally parallel direction to the path of the filaments. The cellulose solution, which is ejected through the orifices, is formed to liquid strands or latent filaments, which are drawn (or significantly decreased in diameter and increased in length and may be split into several sub-filaments) by the gas stream.

The filaments are then collected, for example on a rotating drum, whereby a web is formed.

In the following, this process is referred to as "Lyocell melt-blown process". Nonwoven melt-blown webs made by the Lyocell melt-blowing process will in the following be referred to as "Lyocell melt-blown webs". For the purposes of the present invention, the term "Lyocell melt-blowing process" encompasses both processes by which endless filaments are obtained (such processes also referred to in the literature as "spunbonding processes"), processes by which fibers of a discrete length are obtained and processes by which mixtures of endless filaments and fibers of discrete length are obtained.

In contrast thereto, WO 06/035458 discloses a process for the production of so-called "spunlaid nonwovens", i.e. the extruded filaments are not stretched by a gas stream, but by the flow of the precipitation fluid.

Various means of bonding nonwoven webs are known nowadays. These means, depending on the nature of the nonwoven web employed, comprise chemical bonding, thermal bonding, needle-bonding and bonding via hydroentanglement.

**SUMMARY OF THE INVENTION**

It has now been found that by combining a Lyocell melt-blown process with a hydroentanglement step, it is possible to produce bonded webs with excellent properties for a vari-

## 2

ety of end-uses, with the additional advantage of various synergistic effects, as shown below.

**DETAILED DESCRIPTION OF THE INVENTION**

Hence, one aspect of the present invention relates to a process for the production of a hydroentangled product comprising cellulose fibers, comprising the steps of

(a) extruding a solution comprising cellulose dissolved in an aqueous tertiary amine-oxide through a spinneret into an air gap, thereby forming filaments

(b) drawing said filaments by means of a gaseous stream

(c) collecting and precipitating said filaments in order to form a web

(d) bonding said web by means of a hydroentanglement process

(e) contacting said filaments in the air gap with a medium which at least partially coagulates the filaments.

The inventive process, thereby, is characterized by combining the steps of producing a Lyocell melt-blown web and then bonding said web by means of a hydroentanglement process. Thereby, stable light weight webs resulting from the melt-blown process can be further processed into a bonded web in an especially convenient way.

Step (e) refines the process of step (b) by treating the filaments in the air gap with a partially coagulating medium. Treating the filaments in the air gap with a vapor mist is known, for example, from WO 99/64649.

By way of step (e), the filaments are at least partly precipitated before forming a web. It has been shown that this measure imparts to the webs thusly produced a more soft and textile-like performance, as compared with the more "paper-like" performance of products which are formed by coagulation of the web only after forming the web.

It is, furthermore, believed that by at least partly precipitating the filaments before forming a web, the filaments in the web do not stick together in the same degree as in a web which is formed before precipitating the filaments (non-precipitated filaments spun from a dope of cellulose in NMMO are quite sticky). This facilitates and enhances the effect of the hydroentanglement step (d). This is because for a hydroentanglement step to work effectively, individual filaments should be free to move within the web, i.e. they should not be fused at overlaps.

The medium used in step (e) may preferably be a vapor mist, preferably an aqueous mist.

In a preferred embodiment, step (d) of the process according to the invention is performed on a never-dried web. Under "never-dried web", one understands a web which, after having been formed by collecting and precipitating the filaments, has not yet been dried.

This embodiment brings with it various synergistic effects. In previous processes, first a fiber web was produced which (if produced by a wet route) had to be dried and provided to an external hydroentanglement facility in the dried state.

By combining the melt-blown process and hydroentanglement step without prior drying of the product, both energy, previously needed for drying the original web, and water (previously needed to re-wet the product) can be saved.

Furthermore, as known as such, in the Lyocell process residual solvent must be washed out by aqueous washing liquids. The hydroentanglement step, employing mostly water as the treatment liquid, therefore may act as a further efficient washing step in addition to any prior washing steps, thereby reducing the amount of washing otherwise needed to wash the web.

The preferred embodiment of carrying out the hydroentanglement step on a never-dried web will in the following be referred to as "Online-bonding".

The process according to the invention may further comprise the step of

(f) treating said web by a treatment selected from the group consisting of embossing, perforating and marking the web.

Means to emboss, perforate or otherwise mark a web (such as by applying colored patterns or the like) are known as such to the skilled artisan. It is possible to perform step (f) on a bonded web, that has already been bonded previously.

In a preferred embodiment, step (f) is performed together with step (d). For example, by varying the water pressure during the hydroentanglement step, such as by periodical variation or by variation of the high pressure in different parts across the web marking effects and different densities of the webs, creating an embossed impression, may be achieved.

A further embodiment of the process according to the invention comprises the step of

(g) admixing a further material to either of the solution comprising cellulose dissolved in an aqueous tertiary amine-oxide, a precursor thereof and/or said web.

Under "precursor", any starting or intermediate product of the Lyocell process is meant, such as e.g. the cellulose pulp used for making the solution, the NMNO solvent, a suspension of the pulp and the NMNO solvent used as an intermediate product before making the solution, etc.

Said further material may preferably selected from the group consisting of cellulosic materials, such as cellulosic fibers and pulp, e.g. fluff pulp; non-cellulosic polymers, especially non-cellulosic polymer fibers, bi-component fibers; modifying substances, such as dyestuffs, antibacterial products, ion-exchanger products, active carbon, nanoparticles, lotions, fire-retardant products, superabsorbers, impregnating agents, dyestuffs, finishing agents, crosslinking agents, grafting agents, binders; and mixtures thereof.

Under "binder", an agent being capable of further bonding the web e.g. by thermosetting is meant.

The skilled artisan is well aware which of the above-referenced materials may be added in which step of the Lyocell melt-blown process, and in which manner.

Especially, step (g) may be conducted before step (d). Hence, modifying materials are added to the web or its precursors before the bonding step. After bonding of the web, the materials are more intimately incorporated in the web as compared to a process wherein the materials are added only after bonding of the web.

Said further material can also be admixed to the web by dissolving or dispersing said material in the hydroentanglement fluid employed in step (d). This means, that e.g. a modifying material is added to the hydroentanglement fluid and is incorporated into the web at the same as the bonding via hydroentanglement takes place.

A further embodiment of the process according to the invention comprises the step of

(h) attaching to said web on one or both sides a layer of a further material, especially a fiber-, film- or web-layer.

With this embodiment, it is possible to produce composite materials made up by e.g. one layer of the cellulosic web produced according to the invention and one or more additional layers on one or both sides of the web. "Sandwich" constructions, wherein the cellulosic web is embedded between two, optionally different, layers of e.g. a film or web-like material, are possible.

Said layer may essentially consist of a material selected from the group consisting of cellulosic materials, such as cellulosic fibers and pulp; non-cellulosic polymers; and mixtures thereof.

Examples of composite or "sandwich" products include composites with layers of synthetic polymers, cellulosic fluff pulp, nonwoven webs of cellulose or synthetic polymer fibers, bicomponent fibers, webs of cellulose pulp, such as airlaid pulp, webs or fabrics of high tenacity fibers, hydrophobic materials, high performance fibers (such as bullet proof materials, temperature resistant materials or flame retardant materials, layers imparting changed mechanical properties to the final products (such as Polypropylene or Polyester layers), biodegradable materials (e.g. films, fibers or webs from Polylactic acid), and/or high bulk materials (such as polyacrylnitrile).

Furthermore, it is possible to produce composites where one layer of e.g. a synthetic polymer material is embedded between two or more layers of cellulosic webs produced according to the invention. For example, a sandwich construction with a strong, but physiologically non pleasing, e.g. hydrophobic layer embedded between two cellulosic web layers may be produced. A further example is a sandwich product comprising a layer of airlaid pulp with one or two layers of cellulosic melt-blown web.

Other alternatives comprise composites such as for diapers or sports applications, where, depending on the requirements of the products, either a hydrophilic or a hydrophobic layer is to be in contact with the skin.

In one embodiment of the present invention, step (h), i.e. attaching one or more layers to the cellulosic web, is conducted before step (d).

Especially, it is possible to produce a melt-blown Lyocell web, contacting this web with a layer of e.g. a polymeric fiber material, and then strengthening the composite material by the hydroentanglement step in step (d).

It is also possible to combine several layers of Lyocell melt-blown webs.

To produce various "sandwich" constructions, it is possible to arrange several extrusion heads for extruding the cellulose solution in NMNO, thereby producing several layers of cellulosic melt-blown webs and to suitably arrange sources of additional layers, such as film, fibre or web layers such as to contact the various layers in the desired order, finally obtaining a "sandwich" product with the desired composition of different layers.

Such additional source of an additional layer may as well be an extrusion head for producing a melt-blown or spun-laid product of a synthetic polymer fiber material.

For example, a source for a polypropylene non-woven web can be combined with a source of a Lyocell melt-blown web in such a way that the non-woven polypropylene web is fed onto the never-dried Lyocell melt-blown web. The combined web may then be hydroentangled.

All this can be accomplished "online", i.e. in the framework of the Lyocell melt-blown process, with the preferred option to strengthen the composite so obtained "online" via hydroentanglement step (d).

If nonwoven webs are used as a further layer, these may be pre-bonded or not yet bonded. If such web is not yet bonded, it may be bonded by means of hydroentanglement step (d).

Furthermore, a non-woven waste material may be combined with the melt-blown Lyocell web, e.g. as an additional layer, or by employing a fabric comprising strips of a non-woven waste material woven into said fabric, as e.g. proposed in WO 04/53216.

The use of bicomponent fibers, being incorporated in the cellulosic web and/or being part of one or more of the layers attached thereto, respectively, enables the production of products with a defined ratio of machine direction (MD) to cross direction (CD) orientation, such as e.g. known from WO 03/56088.

The ways to conduct a hydroentanglement treatment on a web of cellulose fibers are known as such to the skilled artisan.

As an example, a Lyocell melt-blown web may be bonded using a spunlace line with 3 pressure heads, the first head operating at around 20 bars, the second head operating at the upper side at around 100 bar and the third head operating at the lower side at around 100 bar. The line speed may be around 40 m/min. If the hydroentanglement step is conducted in an overall continuous process on a never-dried Lyocell melt-blown, the production speed of the spunlace line can be adjusted according to the rate of supply of the web.

After step (d), the bonded web may be further washed, dried, and collected to rolled goods.

In a further aspect, the present invention is directed to a hydroentangled melt-blown web comprising cellulose fibers, obtainable according to the process of the invention.

Hydroentangled melt-blown webs comprising cellulose fibers, especially Lyocell fibers, have not yet been proposed so far. Such webs have excellent properties, rendering them suitable for a variety of possible end-uses.

Typically, a hydroentangled melt-blown web according to the invention may exhibit a weight of 10 g/m<sup>2</sup> to 250 g/m<sup>2</sup>, preferably 30 g/m<sup>2</sup> to 150 g/m<sup>2</sup>, especially preferred 50 g/m<sup>2</sup> to 120 g/m<sup>2</sup>.

The web according to the invention may be present in a perforated, embossed and/or marked state.

In one embodiment of the present invention, the web essentially consists of cellulose.

In an alternative embodiment, the web according to the present invention contains a further material selected from the group consisting of cellulosic materials, such as cellulosic fibers and pulp; non-cellulosic polymers, especially non-cellulosic polymer fibers, bi-component fibers; modifying substances, antibacterial products, ion-exchanger products, nanoparticles, lotions fire-retardant products, absorbency-improving additives, such as superabsorbent resins, carbon resins such as active carbon, graphite, carbon for electrical conductivity; X-ray contrast resins, luminescent pigments, dyestuffs, resins for improvement of the chemical and mechanical stability, finishing agents, crosslinking agents, grafting agents, bonding agents; and mixtures thereof.

Yet one further aspect of the present invention relates to an article containing a web according to the present invention, wherein said web has attached to one or both sides thereof a layer of a further material, especially a fiber-, film- or web-layer.

As already described above, said layer may essentially consist of a material selected from the group consisting of cellulosic materials, such as cellulosic fibers and pulp; non-cellulosic polymers, especially non-cellulosic polymer fibers, bi-component fibers; and mixtures thereof.

The web and the article according to the present invention may be used as a product selected from the group consisting of wipes, filters, absorbent hygiene products, medical products, geotextiles, clothing, building products, automotive products, furnishings, industrial products, leisure and travel products, school and office products; or as a part of such product.

Especially the web and/or the article according to the present invention may be used in a product selected from the

group consisting of wipes, such as baby wipes, kitchen wipes, wet wipes, cosmetic wipes, hygiene wipes, cleaning wipes, glass wipes, lens cleaning wipes, polishing wipes, e.g. for cars and furniture, dust wipes, industrial wipes, intimate 5 wipes, toilet wipes, floor wipes, glass wipes, medical wipes, such as cleansing and pre-operative wipes, dusters and mops; filters, such as air filters, e.g. HVAC, HEPA and ULPA filters, flue gas filters, liquid filters, coffee filters, tea bags, coffee bags, food filters, water purification filters, blood filters, cigarette filters, cabin filters, fuel filters, oil filters, cartridge filters, vacuum filters, vacuum cleaner bags, dust filters, hydraulic filters, kitchen filters, fan filters, beer filters, milk filters, liquid coolant filters, fruit juices filters, face masks and active carbon filters; disposable absorbent products such as acquisition layers, coverstock, distribution layers, absorbent covers, sanitary napkins, panty liners, diapers, incontinence products, towels, tampons, sanitary pads, backsheets, leg cuffs, flushable products, pads, nursing pads, disposable underwear, training pants, cosmetic removal pads and washcloths; medical products, such as disposable caps, gowns, masks and shoe covers, wound care, sterile packaging, coverstock, dressing materials, one way clothing, dialysis products, nasal strips, adhesive for dental plates, drapes, wraps and packs, sponges dressing and wipes, bed linen, transdermal drug delivery, shrouds, underpads, procedure packs, heat packs, ostomy bag liners, fixation tapes and incubator mattresses; structural and/or reinforcement products such as geotextile products, capillary matting, water purification products, irrigation control products, asphalt overlay, soil stabilization products, drainage products, e.g. drainage channel liners, sedimentation and erosion control products, pond liners, impregnation base products, ground stabilization products, pit linings, seed blankets, weed control fabrics, greenhouse shading, root bags and biodegradable plant pots; 30 building products, such as roofing and tile underlay, underlating, thermal and noise insulation, house wraps, facings for plaster board, pipe wraps, concrete molding layers, foundations and ground stabilization products, vertical drainages, shingles, roofing felts, noise abatement materials, reinforcement materials, sealing materials, mechanical damping materials, fire protection materials, support material for bitumen coating, reinforced concrete and reinforced polymers; automotive products, such as cabin filters, boot liners, parcel shelves, heat shields, shelf trim, molded bonnet liners, boot 35 floor covering, oil filters, headliners, rear parcel shelves, decorative fabrics, airbags, silencer pads, insulation materials, car covers, underpadding, car mats, tapes, backing and tufted carpets, seat covers, door trim, needled carpets, auto carpet backings, and reinforced polymers; furnishing products, such as furniture constructions, insulators to arms and backs, cushion thickings, dust covers, linings, stitch reinforcements, edge trim materials, bedding constructions, quilt backing, spring wraps, mattress pad components, mattress covers, window curtains, wall coverings, carpet backings, lampshades, mattress components, spring insulators, sealings, pillow thickening, mattress thickening and high loft webs for filling applications such as disposable duvets; industrial products, such as electronic products, floppy disc liners, cable insulation, abrasives, insulation tapes, conveyor belts, noise 40 absorbent layers, air conditioning products, battery separators, acid systems, anti slip matting, stain removers, food wraps, adhesive tapes, sausage casings, cheese casing, artificial leather, oil recovery booms and socks, papermaking felts, kettle descaler bags, and flame barriers; travel or leisure products, such as sleeping bags, tents, luggage, handbags, shopping bags, airline headrests, CD-protection products, pillow-cases, sandwich packaging and surf boards; and school or 45

office products, such as book covers, mailing envelopes, maps, signs and pennants, towels, flags and bank notes; or as part of such product.

What is claimed is:

1. A process for the production of a hydroentangled product comprising cellulose fibers, comprising the steps of
  - (a) extruding a solution comprising cellulose dissolved in an aqueous tertiary amine-oxide through a spinneret into an air gap, thereby forming filaments,
  - (b) drawing said filaments by means of a gaseous stream,
  - (c) collecting and precipitating said filaments in order to form a web,
  - (d) bonding said web by means of a hydroentanglement process, and
  - (e) contacting said filaments in the air gap with a medium which at least partially coagulates the filaments, wherein step (d) is performed on a never-dried web.
2. The process according to claim 1, wherein said medium is selected from the group consisting of a vapor mist and an aqueous mist.
3. The process according to claim 1, further comprising the step of
  - (f) treating said web by a treatment selected from the group consisting of embossing, perforating and marking the web.
4. The process according to claim 3, wherein step (f) is performed on a previously bonded web.
5. The process according to claim 3, wherein step (f) is performed together with step (d).
6. The process according to any of the preceding claims, further comprising the step of
  - (g) admixing a further material to either of the solution comprising cellulose dissolved in an aqueous tertiary amine-oxide, a precursor thereof and/or said web.
7. The process according to claim 6 wherein said further material is selected from the group consisting of cellulosic materials, non-cellulosic polymers, modifying substances,

antibacterial products, ion-exchanger products, active carbon, nanoparticles, lotions, fire-retardant products, superabsorbers, impregnating agents, dyestuffs, finishing agents, crosslinking agents, grafting agents, binders, and mixtures thereof.

8. The process according to claim 6, wherein step (g) is conducted before step (d).
9. The process according to claim 6, wherein said further material is admixed to the web by dissolving or dispersing 10 said material in the hydroentanglement fluid employed in step (d).
10. The process according to claim 6, further comprising the step of
  - (h) attaching to said web on one or both sides a layer of a further material.
11. The process according to claim 10, wherein said layer comprises a material selected from the group consisting of cellulosic materials, non-cellulosic polymers, and mixtures thereof.
12. The process according to claim 10, wherein step (h) is conducted before step (d).
13. The process according to claim 7, wherein the cellulosic materials are selected from the group consisting of cellulosic fibers and pulp.
14. The process according to claim 7, wherein said non-cellulosic polymers are selected from the group consisting of non-cellulosic polymer fibers and bi-component fibers.
15. The process according to claim 10, wherein said further material is selected from the group consisting of a fiber-layer, 30 a film-layer and a web-layer.
16. The process according to claim 11, wherein said cellulosic materials are selected from the group consisting of cellulosic fibers and pulp.
17. The process according to claim 11, wherein said non-cellulosic polymers are selected from the group consisting of 35 non-cellulosic polymer fibers and bi-component fibers.

\* \* \* \* \*